

## UNITED STATES PATENT OFFICE

2,099,347

## RECOVERY OF CELLULOSE ESTERS FROM SCRAP

Marvin J. Reid, Rochester, N. Y., assignor to  
Eastman Kodak Company, Rochester, N. Y., a  
corporation of New Jersey

No Drawing. Application February 10, 1937,  
Serial No. 125,116

8 Claims. (Cl. 260—102)

This application relates to the recovery of an organic acid ester of cellulose which has been used as the base for photographic film from the scrap film by means of a mixture of acetone and a lower 5 aliphatic alcohol.

Photographic film is composed of a photosensitive gelatin emulsion supported by a reenforcing layer commonly referred to as the film base. Often the film base needs to be overcoated or 10 subbed with a layer of material to promote the adhesion of the photosensitive emulsion thereto. Also, with some types of film it is desirable that the base or the subbing layer or both be tinted to give desired effects or to prevent halation or both. 15 When photographic film is scrapped, it is desirable to recover the organic acid ester of cellulose, which is used as the base of the film. To do this requires the removal of the photosensitive emulsion and of the subbing layers and the tinting 20 material which has been employed therewith. In some cases additional layers are put on, such as to still further increase the adhesiveness of the emulsion to the film base.

Various methods have been proposed for removing these additional materials which are employed with a film base to prepare photographic film. For instance, for the removal of the color 25 from tinted film the combination of bleaching and washing has been suggested, however, by this process small amounts of impurities are left in the film support which are injurious to some types of photosensitive emulsions and, therefore, the use 30 of the scrap, recovered by this means, is restricted.

I have found that a mixture of acetone and an 35 aliphatic alcohol, consisting predominately of the latter, is eminently suited to the removal of the subbing layers used on film base comprising substantially complete removal of the tinting material 40 from a tinted film base. A mixture, which has been found to be generally suitable, consists of 85% of the lower aliphatic alcohol particularly methyl alcohol and 15% acetone, although the proportion of acetone may range from 10-20% 45 and still form a leaching liquid which is quite satisfactory.

The subbing material which is commonly employed on film base consisting of an organic acid ester of cellulose is either a resin of the synthetic 50 type, such as a bakelite resin or one of the polyvinyl resins or an organic acid ester of cellulose which has been hydrolyzed much further than the organic acid ester of cellulose which is employed for the film base. As an example of recovering 55 the ester from scrap film, the scrap is comminuted

and washed with warm water to remove the emulsion and any gelatin coatings thereon. It is then leached with a mixture of the alcohol and acetone, preferably in a counter-current system. After the subbing layers and tinting have been 5 sufficiently removed, the scrap is then washed with water to thoroughly remove the solution and recover it from the scrap. The support is then dried and kept stored for future use in the preparation of solutions for making colloidized products. Obviously, if the base is made from an 10 ester which has been hydrolyzed considerably, the acetone-alcohol mixture might soften the base to too great an extent. At the present time, however, the film base, which is ordinarily used, is of 15 a type which will not be affected by the alcohol-acetone mixture and, therefore, my invention is eminently suited for the recovery of that type of film. The organic acid ester of cellulose subbing 20 layers may be composed of either hydrolyzed cellulose acetate, cellulose acetate propionate or cellulose acetate butyrate which has been hydrolyzed considerably beyond the point where the hydrolysis to obtain an ester suitable for making the film base is usually stopped.

In photographic film the subbing layer and the tint join themselves very closely to the film base and almost seem to penetrate into the pores thereof. Therefore, a rather severe treatment is necessary to remove the tinting material and the 25 hydrolyzed ester which has been employed as the sub. I have found that by the incorporation of a small amount of acetone, the mixture formed is especially adapted to rendering the impurities 30 more susceptible to removal by the leaching solvent, particularly as the acetone seems to exert 35 a swelling action on the film base.

The following examples illustrate the application of my invention to different types of photographic film scrap.

*Example I*

Approximately 250 pounds (dry weight) of photographic film scrap, having a base of cellulose acetate and a subbing layer of a cellulose 45 acetate which has been hydrolyzed to 25-30% acetyl, was chopped into pieces about 2 in. square and then soaked in warm water at 110° F. for 24 hours and was then washed in several changes of warm water at 110° F. The scrap was then 50 leached in an agitated jacketed vessel using three one hour changes of a solution of methyl alcohol-acetone (85:15) at 80-100° F. The scrap was wet when treated with the mixture, however, in the first treatment the amount of water pres- 55

ent was not more than 30% while with the second step, the amount of water was below 15% and for the third step, the water had decreased to 5%. These water contents are the most that 5 can be tolerated in the process, hence it is undesirable to use scrap which is in too wet a condition. The solvent was used counter-currently 10 on successive batches in order to make for economical operation of the process. After the 15 third treatment, the recovered scrap was separated from the leaching liquid and thoroughly washed with water to remove the solvent after which it was dried. As a matter of economy, it is also desirable to carry out the washing of the 20 scrap with water in a counter-current system. After the recovered scrap is dried, it can be stored and employed in making up solutions alone or with additional fresh material.

#### Example II

20 Approximately 250 pounds of photographic film scrap, having a film base of cellulose acetate and a subbing layer of a Bakelite resin, was comminuted and washed with warm water to remove 25 the emulsion therefrom. It was then leached with three one hour changes of methyl alcohol-acetone (85:15) at approximately 80° F. The scrap was leached in approximately 750 gals. of 30 solution. The recovered scrap was then washed and dried, as pointed out in Example I. Instead of 80° F., a temperature of 80°-100° F., or even more, would be quite satisfactory.

Instead of the subbing layer being of a Bakelite resin, it may be of some other synthetic resin. Both the subbing layer and the tinting material, if any is present, is removed by this 35 treatment.

#### Example III

40 Cellulose acetate film support subbed with gelatin containing a blue dye and coated with an emulsion was chopped into small pieces and washed in warm water to remove the emulsion and gelatin coatings therefrom. The dye had 45 penetrated the cellulose acetate base and this dye was not removed by the warm water washing. About 500 pounds of this wet, washed film scrap was added to 750 gals. of methyl alcohol-acetone (85:15) and the mass was agitated for 50 one hour while maintaining a temperature of 100° F. The solution was withdrawn and the scrap was again treated with a second 750 gals. of a like mixture of methyl alcohol and acetone, being agitated for the same time and at the same 55 temperature. This treatment was repeated making three one hour treatments in all. The scrap was then washed in several changes of water and was then dried and stored for use in making cellulose acetate dope solutions.

60 The solution of methyl alcohol and acetone softens and swells the support at 100° F. sufficiently so that the tinting material can be satisfactorily removed therefrom but not to such 65 a degree that the scrap cannot be safely agitated. This swelling and softening can be controlled by varying the temperature of the solution so that, if the removal of the tinting material is not as complete as desirable, the temperature may be 70 greater, while if the solvent is causing so much swelling that the scrap will not stand up after agitation in the solution, a temperature of less degree is then desirable for maximum results.

75 My invention is not limited to the use of methyl alcohol as other lower aliphatic alcohols

may be employed in admixture with acetone to recover film scrap. Ethyl alcohol may be employed as the lower aliphatic alcohol in which case it is preferable that more acetone be employed to give sufficient swelling action. This is 5 because ethyl alcohol alone appears to have practically no swelling action on cellulose acetate or the other organic acid esters of cellulose.

Mixtures of isopropyl alcohol and acetone are 10 very satisfactory for the recovery of organic acid esters of cellulose from scrap film. Butyl alcohol-acetone might be employed but has the disadvantage of the low solubility of the butyl alcohol in water. As the water insolubility of 15 the alcohols increases beyond the alcohols of 4 carbon atoms this point may be considered the practical limit of the alcohol constituent.

20 My process is applicable to the usual type of film base prepared from the lower fatty acid esters of cellulose, such as cellulose acetate or cellulose acetate propionate or acetate butyrate. Obviously, if the ester employed in preparing the film base should be so susceptible to the action of the methyl alcohol-acetone mixture that 25 it softens to an appreciable degree, my process would not give the best results therewith, although it could be employed.

30 In addition to the subbing layers and the tinting materials which are employed in the photographic films with the cellulose esters, plasticizers are also usually present. My recovery process has the advantage that it also removes 35 practically all of the plasticizer from the ester. Also, if nitrocellulose subbing layers are present in the scrap film, that material is also removed 40 in my process for recovering film scrap.

I claim:—

45 1. A method for recovering photographic film having a base of a lower organic acid ester of cellulose which comprises washing the film scrap with warm water, then leaching it with a mixture of a lower aliphatic alcohol and acetone, in proportions which will swell the cellulose ester, at a temperature of 68°-110° F. under conditions whereby the scrap is not greatly softened 45 and then washing the scrap to remove the leaching solution therefrom.

50 2. A method of recovering photographic film having a cellulose acetate base which comprises washing the film scrap with warm water, then leaching it with a mixture of a lower aliphatic alcohol and acetone, in proportions which will swell the cellulose acetate, at a temperature of 68°-110° F. under conditions whereby the scrap 55 is not greatly softened and then washing the scrap to remove the leaching solution therefrom.

55 3. A method for recovering photographic film scrap having a base of a lower organic acid ester 60 of cellulose which comprises washing the film scrap with warm water, then leaching it with a mixture of methyl alcohol and acetone containing 10-20% of the latter, at 68°-110° F. under conditions whereby the scrap is not greatly softened, then washing the scrap to remove the 65 leaching solution therefrom.

70 4. A method for recovering photographic film scrap having a base of a lower organic acid ester 70 of cellulose which comprises washing the film scrap with warm water, then leaching it with a mixture of isopropyl alcohol and acetone containing 10-20% of the latter, at 68°-110° F. under conditions whereby the scrap is not greatly 75

softened, then washing the scrap to remove the leaching solution therefrom.

5. A method for recovering photographic film scrap having a cellulose acetate base which comprises washing the film scrap with warm water, then leaching it with a mixture of methyl alcohol and acetone containing 10-20% of the latter, at 68°-110° F. under conditions whereby the scrap is not greatly softened and then washing 10 the scrap to remove the leaching solution therefrom.

6. A method for recovering photographic film scrap having a cellulose acetate base which comprises washing the film scrap with warm water, then leaching it with a mixture of isopropyl alcohol and acetone containing 10-20% of the latter, at 68°-110° F. under conditions whereby the scrap is not greatly softened and then wash-

ing the scrap to remove the leaching solution therefrom.

7. A method for recovering photographic film scrap having a base of a lower organic acid ester of cellulose which comprises washing the film 5 scrap with warm water, then leaching it with a mixture of a lower aliphatic alcohol and acetone, in proportions which will swell the cellulose ester, at a temperature of 68°-110° F. under conditions whereby the scrap is not greatly sof- 10 tened.

8. A method for recovering photographic film scrap having a cellulose acetate base which comprises washing the film scrap with warm water, then leaching it with a mixture of methyl al- 15 cohohol and acetone containing 10-20% of the latter, at 68°-110° F. under conditions whereby the scrap is not greatly softened.

MARVIN J. REID.